

## UNITED STATES PATENT OFFICE

WILLIAM F. GEHRIG, OF BERKLEY HEIGHTS, NEW JERSEY, ASSIGNOR TO ESSEX SPECIALTY CO., INC., OF BERKLEY HEIGHTS, NEW JERSEY, A CORPORATION OF NEW JERSEY

## DETONATING FIREWORK COMPOSITION

No Drawing.

Application filed March 12, 1929. Serial No. 346,498.

This invention relates to fireworks which are set in action by means of impact, or friction, or heat, and which during combustion thereof produce a succession of explosive detonations or reports, the action taking place in such manner that the article does not explode in mass but burns with relatively slow combustion accompanied by rapid intermittent, small and harmless explosions. 5 Heretofore, such form of fireworks have been made with poisonous yellow phosphorus, potassium chlorate and an organic binding material, such as shellac or gum.

In order to avoid the use of the poisonous yellow phosphorus, it has been proposed to employ sulphur phosphorous compounds and particularly sesquisulphide of phosphorus as the active agent with an oxygen producing element in the form of potassium chlorate, 20 the compound being bound in intimate mixture by a cementitious binder comprising magnesium chloride and magnesium oxide. It has been found, however, that such form of binder is not altogether satisfactory for 25 the reason that the magnesium chloride ingredient thereof being very hygroscopic, the finished article is sensitive to climatic changes, tending to crumble and deteriorate especially in damp or humid weather.

30 In my copending application, Serial No. 238,467 filed December 7, 1927, there is disclosed a firework composition that produces a succession of explosive detonations or reports during combustion and which is not sensitive to moisture and is non-hygroscopic.

It is the primary object of the present invention to provide an improved composition of the kind described in my above mentioned application which composition is non-poisonous and not sensitive to moisture and which therefore will not readily deteriorate under changing climatic or weather conditions, but will remain firm and hard at all times so as to be properly operative when put to the 40 use for which it is intended; and to this end

use is made of binder and hardening ingredients of the composition comprising a mixture of alum such as chrome alum and metallic oxides, for example magnesium oxide and ferric oxide. This composite binder and 50 hardening agent of this invention is non-hygroscopic, and produces a hard inorganic cementitious material or carrier through which the phosphorous sesquisulphide and oxygen producing materials may be dispersed and 55 retained in that closely incorporated relation necessary to effect the character of combustion producing the successive or intermittent small explosions or reports rather than relatively slow flaming and free burning combustion which it is desired to avoid. 60

Another object of the present invention is to provide a firework composition which will give a maximum number of intermittent detonations during the combustion thereof. 65

In order to obtain the greatest number of intermittent detonations from a given mass of composition, a dispersive agent is used in sufficient quantity to facilitate the complete and uniform dispersion of the phosphorus 70 sesquisulphide particles throughout the mass of the composition. An aqueous solution of a suitable gum such as gum arabic is employed as the dispersive agent, the amount of gum used being just sufficient to facilitate 75 the dispersion so as to place the composition in a colloidal state, the various ingredients thereof being held in mechanical suspension by the aqueous gum solution. The phosphorus sesquisulphide so dispersed is distributed throughout the mass of the composition and each particle separated from other particles thereof by the composite binder and 80 hardening agent which acts to restrain the burning of the material and thereby obtain 85 intermittent detonation.

In making up the novel firework composition of this invention, an aqueous solution of gum arabic is introduced in a water mixture of chrome alum to which has been added fer- 90

ric oxide, potassium chlorate and phosphorus sesquisulphide. To this mixture is added magnesium oxide, whereupon the mixture is then formed into discs or other shapes or spread on a suitable surface and dried.

5 As an example of the composition of this invention, the ingredients are mixed together in the following proportions by weight:—

|                              | Parts |
|------------------------------|-------|
| 10 Potassium chlorate        | 25    |
| Magnesium oxide              | 35    |
| Chromium potassium sulphate  | 5     |
| Sesquisulphide of phosphorus | 8     |
| Ferric oxide                 | 5     |
| 15 Gum arabic                | 2     |

The preferred manner of preparing the composition is as follows:—

Two pounds of gum arabic is dissolved in cold water and allowed to stand for about a 20 day. Five pounds of chrome alum (chromium potassium sulphate) is placed in a mixer and sufficient cold water is added to completely dissolve the same. Five pounds of ferric oxide is then mixed into the chrome alum solution and then twenty five pounds of potassium chlorate is also mixed into this solution. To this mixture, eight pounds of sesquisulphide of phosphorus preferably in granulated form is then added and intermixed therewith. To the resultant mixture of chrome alum, ferric oxide, potassium chlorate and phosphorus sesquisulphide is added the previously prepared gum arabic solution. Thirtynine pounds of magnesium oxide is then added and the resulting mixture thoroughly agitated until all materials are in a colloidal state, the gum arabic solution acting to hold the other ingredients in mechanical suspension. After the paste is thus produced, it is placed under slight pressure in molds and then allowed to dry over night at a temperature varying from 80 to 90 degrees Fahrenheit, or the paste may be deposited on paper strips or sheets in the form of segregated spots or pellets, or the paste may be deposited on a fuse material; in any case when dried the same will provide a combustible composition which, when ignited will burn in such manner as to produce the desired series of rapid succession of detonations or explosions.

50 The composition thus produced, will, when dried, provide a relatively hard dense mass which is non-hygroscopic so that it keeps well under variations of climatic or weather conditions, is not subject to spontaneous combustion, and will remain properly operative for the purposes intended. The hardening of the composition is due to the interaction of 55 the composite binder constituents. During and after the drying process, the chrome alum evidently reacts in the proportions given with the magnesium and ferric oxides to form metallic oxy-sulphates which are of considerable hardness and are similar in characteris-

tics to the metallic oxy-chlorides which are present in certain cements. These metallic oxy-sulphates render the composition hard and resistant to moisture and also aid in separating particles of phosphorus sesquisulphide so as to thereby restrain the burning of the material and obtain intermittent detonation. Any excess of oxides merely serves as a filler. The potassium chlorate furnishes oxygen to support the combustion after ignition has taken place.

70 The composition of the kind described possesses, in addition to the keeping qualities above mentioned, a thorough dispersion of the phosphorus sesquisulphide, a tenacious adhesion of all constituents of the composition one to the other owing to the cementing action of the composite binder, and the highly desirable advantage of being free from poisonous substances.

75 While in the above illustrative table there is given the relative proportions of the several ingredients of the composition, it will be understood that variation of the stated proportions may be made within reasonable limits. For example, by increasing the relative proportion of potassium chlorate with proportionate decrease of magnesium and ferric oxides and chrome alum, the action of the firework will be speeded up, i.e. the combustion thereof accompanied by the detonations will be more rapid; while, on the other hand, by decreasing the relative proportion of potassium chlorate with proportionate increase in magnesium and ferric oxides and chrome 80 alum, the action of the firework will be slowed down, i.e. the combustion thereof accompanied by the detonations will be slower. Changes in the balance of the other ingredients within reasonable limits may be also 85 made while still attaining the purposes and function of the composition within the scope and spirit of this invention.

90 It will be noted that the composition of the instant invention is to be distinguished from the composition in my aforesaid copending application in that the inclusion of the gum ingredient serves to produce a better and more uniform dispersion of the phosphorus compound and the oxygen supplying agent, particularly since the gum solution acts to put the composition in a colloidal condition wherein the ingredients above mentioned are more thoroughly and uniformly dispersed and segregated in small particles or globules throughout the mass of the mixture. For this reason, the composition of the instant invention may be considered a specific improvement over my copending application and a 95 development of the latter serving to produce a better composition from a manufacturing and commercial standpoint.

100 Having thus described the invention, what is claimed is:—

1. A non-hygroscopic firework composi-

tion adapted to produce successive detonations when ignited, comprising at least one sulphur-phosphorus compound as its active agent, at least one chlorate for producing oxygen, a composite binder comprising a metallic oxide and an alum, and gum as a dispersive agent.

2. A non-hygroscopic firework composition adapted to produce successive detonations when ignited, comprising at least one sulphur-phosphorus compound as its active agent, at least one chlorate as the oxygen producing substance, an inorganic binder consisting in magnesium and ferric oxides and an alum, and gum as a dispersive agent.

10 3. A non-hygroscopic firework composition adapted to produce successive detonations when ignited, comprising a mixture of the herein named ingredients in approximate proportions as follows:

|                              | Parts |
|------------------------------|-------|
| Potassium chlorate           | 25    |
| Magnesium oxide              | 35    |
| Chromium potassium sulphate  | 5     |
| Sesquisulphide of phosphorus | 8     |
| 25 Ferric oxide              | 5     |
| Gum arabic                   | 2     |

In testimony, that I claim the invention set forth above I have hereunto set my hand

20 this 28th day of February, 1929.

WILLIAM F. GEHRIG.

35

40

45

50

55

60

65